

## UNITED STATES PATENT OFFICE

1,949,775

## FLUID COMPOSITION

Jules Bebie and George L. Doelling, St. Louis, Mo.,  
 assignors to Wagner Electric Corporation, St.  
 Louis, Mo., a corporation of Delaware

No Drawing. Application June 29, 1932,  
 Serial No. 619,993

3 Claims. (Cl. 252—5)

Our invention relates to a fluid composition suitable for use in fluid pressure devices such as hydraulic actuating apparatus for vehicle brakes and in its more specific aspect constitutes 5 an improvement in the castor oil-alcohol type of fluid now in general use for this purpose, this last mentioned fluid consisting chiefly of castor oil and ethyl alcohol in approximately equal proportions.

10 It is desirable that a hydraulic brake fluid have quite a number of special characteristics, such as very low freezing point; substantially non-volatile at temperatures up to at least 300 degrees Fahr.; without physical or chemical effect 15 upon rubber; non-corrosive to metals, such as copper, brass and steel; have good lubricating properties; and form a film on the metal surfaces of the cylinders over which pistons and 20 piston sealing cups move, which will constitute protection against atmospheric corrosion.

A hydraulic brake fluid consisting of alcohol and castor oil falls short of ideal fulfillment of the above desiderata but does have the important 25 advantage of being relatively inexpensive. We have found that a greatly improved fluid is secured by adding to the alcohol-castor oil mixture a small quantity of a toluene sulfonamid ester. This produces a liquid having a much lower 30 freezing point, less deteriorating effect on rubber, and less corrosion of the metal parts due to the better film which the fluid forms. We have also found that the solidifying point is 35 considerably lowered if, instead of a single toluene sulfonamid ester, substantially equal portions of ethyl ester of ortho toluene sulfonamid and ethyl ester of para toluene sulfonamid are employed.

40 While the proportions may be somewhat varied,

a fluid having the following composition has very satisfactory characteristics:

|                                         | Parts by<br>volume |
|-----------------------------------------|--------------------|
| Castor oil                              | 35                 |
| Ethyl ester of ortho toluene sulfonamid | 10                 |
| Ethyl ester of para toluene sulfonamid  | 10                 |
| Ethyl alcohol                           | 45                 |

A fluid of the foregoing composition does not solidify at temperatures above approximately 65 —40 degrees Fahr. and is of satisfactory viscosity throughout the operating temperature range. Since oils other than castor oil may be suitable for use in the composition, provided they 70 are stable under substantial range of temperature, have low solidifying point, and do not affect rubber, we do not desire that our invention in its broadest aspect be limited to a fluid embodying castor oil as the main lubricating element. 75

Having fully described our invention, what we 75 claim as new and desire to secure by Letters Patent of the United States is:

1. An operating fluid for fluid pressure apparatus comprising alcohol, a toluene sulfonamid ester, and an oil characterized by low solidifying point and inertness toward rubber. 80

2. The combination with a fluid pressure device comprising exposed rubber and metal, of an operating fluid therein comprising castor oil, alcohol, and a toluene sulfonamid ester. 85

3. An operating fluid for fluid pressure apparatus consisting of castor oil in approximately 35 parts by volume, ethyl ester of ortho toluene sulfonamid in approximately 10 parts by volume, ethyl ester of para toluene sulfonamid in approximately 10 parts by volume, and ethyl alcohol in approximately 45 parts by volume. 90

JULES BEBIE.

GEORGE L. DOELLING. 95

40

100

45

100

50

105

55

110